

# United States Patent [19]

Faraci et al.

[11] 3,797,220

[45] Mar. 19, 1974

[54] METHOD FOR THE TEXTURIZATION OF  
YARNS, AND THE PRODUCT THEREOF

[75] Inventors: Giorgio Faraci; Giuseppe Godi, both  
of Gozzana, Italy

[73] Assignee: Bemberg S.p.A., Milan, Italy

[22] Filed: Mar. 16, 1971

[21] Appl. No.: 124,797

[30] Foreign Application Priority Data

Mar. 18, 1970 Italy ..... 22137/70

[52] U.S. Cl. 57/140 R, 57/34 HS, 57/157 TS

[51] Int. Cl. D02g 1/02

[58] Field of Search 57/34 HS, 77.4, 157 TS,  
57/140 R

[56] References Cited

UNITED STATES PATENTS

3,376,698 4/1968 Whittaker et al. .... 57/34 HS  
3,029,591 4/1962 Scragg et al. .... 57/77.4 X

|           |         |                     |           |
|-----------|---------|---------------------|-----------|
| 3,018,609 | 1/1962  | Maier et al. ....   | 57/157 TS |
| 3,069,837 | 12/1962 | Olson .....         | 57/157 TS |
| 3,093,955 | 6/1963  | Cadario .....       | 57/34 HS  |
| 3,474,612 | 10/1969 | Jenkins et al. .... | 57/34 HS  |

Primary Examiner—John Petrakes  
Attorney, Agent, or Firm—Diller, Brown, Ramik & Holt

[57] ABSTRACT

A method and a device for texturing yarns, more particularly synthetic yarns, is disclosed, in which the false twist annular body is made of rubber having a hardness of 70 Shore and over. Advantageously, the yarn is heated, upstream of the false twist annular body, at a temperature well below the melting point of the material forming the yarn. Critical dimensions for the false twist annular body and for the distance therefrom of the tube on which the yarn is wound, are also specified. It is preferred that the yarn be drawn prior to reaching the false twist annular body.

6 Claims, 1 Drawing Figure



PATENTED MAR 19 1974

3,797,220



INVENTORS  
GIORGIO FARACI &  
GIUSEPPE GODI

BY *Dilker, Brown, Pamela & Holt*

ATTORNEYS

## METHOD FOR THE TEXTURIZATION OF YARNS, AND THE PRODUCT THEREOF

This invention relates to a method for the production of a texturized yarn, in which a sliding yarn, while it forms a balloon, is wound around a spindle with the aid of a vertically ring and traveler which surrounds said spindle, in which method the yarn is heated and, as it enters the balloon it rotates about its own longitudinal axis and slides against an annular false-twisting body, so as to impart to the yarn a twist angle. The invention also comprises a device for performing the method and the yarn obtained thereby.

A method as mentioned above is conventional. In the known method the false-twist annular body is also a heating means, so that it is difficult to select an appropriate material for the interior surface of the annular false twist body, that is, the material on which the yarn is allowed to slide in the most regular possible manner. As a matter of fact, a regular sliding of the yarn against said surface is necessary in order that a uniform yarn, having a sufficient degree of false twist, or texturization, may be obtained. Furthermore, in the known method, the annular false-twist body is positioned above the rotating spindle at a rather long distance therefrom.

An object of the invention is to provide a method of the kind referred to above, which is not impaired by the defects enumerated hereinabove. The method according to the invention is characterized in that the surface of the annular false-twist body is made of rubber or another material which has similar frictional properties.

According to a preferred embodiment, the inside diameter of the annular false-twist body varies between 10 mms. greater than and 30 mms. less than the outside diameter of the tube on which the treated yarn is wound, whereas the distance between the lower portion of the annular false-twist body and the upper portion of the tube is between 1 and 10 mms. According to the invention it is preferred that the balloon tension of the yarn is kept virtually constant. This can be obtained by varying the spindle speed according to a pre-selected program.

According to the invention, particularly favourable results are obtained if the yarn is heated upstream of the annular false-twist body, for example by a heated pin, a heated plate or a heated roller, which have a temperature lying in the range from 15°C and 60°C below the melting point of the thread, for example in the case of a polyamide yarn.

According to the invention, the method is advantageously performed if the yarn is drawn upstream of the annular false-twist body, the latter being preferably made of a rubber having a hardness of at least 70 Shore.

A device for performing the method according to the invention comprises yarn feeding means, yarn forwarding means, a ring spindle on which a tube for winding the yarn is inserted, an annular false-twist body placed above said ring spindle, and means for heating the yarn, and is characterized in that the surface of the annular false-twist body over which the yarn slides is of rubber, which more particularly has a hardness of at least 70 Shore, or is of a different material having similar frictional properties.

According to a preferred embodiment of the device according to the invention, a yarn-heating means is provided upstream of the annular false-twist body.

The invention will now be illustrated in more detail with reference to the accompanying diagrammatical drawing.

A non texturized starting yarn 1, which is not drawn, is unthreaded from a spool 2 through a yarn guide 3 placed in front of the spool. The yarn is guided by a 10 guiding roller 4 towards a driven feed roller 5 coupled with a pressure roller 6. Subsequently, the yarn is drawn by a driven drawing roller 7 with the aid of a separator roller 8, the surface speed of the drawing roller being adjusted so as to be a few times a multiple of that 15 of the feed roller. Then the drawn yarn passes over a hot pin 9 and enters the annular false-twist body 10 whose internal surface is of a rubber having a hardness of at least 70 Shore, the body 10 having a height of 30 mms., and inside diameter of 28 mms., and an outside 20 diameter of 48 mms. The yarn slides against the surface of the inner circumference of the false-twist body 10, which is arranged above the tube 11, about which the yarn is wound, at a distance ranging from 1 to 10 mms. The diameter of the tube 11 is 50 mms. The tube 11 is inserted into a driven twisting spindle 12. On the tube 11 the yarn is wound in the form of a pack 13 by means of a vertically reciprocable ring and traveler system 14 which causes the yarn to rotate and to build a balloon 15 between the ring 14 and the annular false-twist body 10. The annular false-twist body is not rotated. However, with the aid of the annular false-twist body 10, a very high degree of false-twist can be imparted to the yarn, inasmuch as the diameter of the yarn is much smaller than the inside diameter of the annular false-twist body over which the yarn is forced to slide.

By way of example, favourable results have been achieved with a 6-filament polycaprolactam yarn having a count of 22 dtex., said yarn having been drawn at a draw ratio of 2.65 and at a surface speed of the drawing roller 7 of 400 meters a minute.

The drawn yarn had the following specifications:

|                      |                        |
|----------------------|------------------------|
| Elongation at break  | 31.5%                  |
| Tensile strength     | 420 gr/100 dtex        |
| Shrinkage            | 71%                    |
| Sensitivity to twist | 209 revolutions/50 cm. |

With the term shrinkage, there is intended herein to indicate a measuring taken according to the following method. A hank of 10 meters of a yarn sample, prepared by winding the aforesaid yarn length on a reel having 1 meter of outside circumference under a tension of 0.1 grams/dtex was immersed during 30 seconds in a bath of water heated to 95°C and then hung on a hook. A weight of 0.2 grams/dtex is then hung to the hank and, after one minute the total length ( $L_1$ ) taken by the hank is read on a dial placed behind the hank. The weight is removed and the shank is transferred during 45 minutes into an oven with air heated to 60°C, whereafter the hank is removed from the oven and placed to be conditioned during 60 minutes in an atmosphere as conditioned to 22°C and 65 percent rel. humidity. After that time, the hank is hung again to the hook and a weight of 0.002 grams/dtex is hung to the hank and the length ( $L_2$ ) taken by the hank is read after one minute.

Shrinkage is calculated with the formula

$$(L_1 - L_2/L_1) \times 100$$

With the term "sensitivity to twist," it is intended

herein to connote a measure taken according to the following method. A section of horizontal yarn is affixed at its two ends to two clamps, so as to have a yarn length comprised between the two clamps of 50 cms. and a tension of the yarn equal to the weight of 1,000 meters of the yarn. A 2-gram weight is hung at the middle of the horizontal yarn length and the two clamps, which can slide on a horizontal plane, are approached until they contact one another. By so doing, the yarn forms a loop which is twisted over itself a certain number of times, inasmuch as the yarn has a twisting moment. Once an equilibrium has been reached, a revolution counter indicates how many revolutions are required to untwist the loop. This value, as referred to the 15 50-cms. length of yarn expresses just the sensitivity to twist.

Variations are possible within the scope of the invention.

What is claimed is:

1. A method for the production of texturized yarn, in which a sliding yarn is wound, as it builds up a balloon, on a spindle with the aid of a vertically reciprocable ring and traveler which surrounds said spindle, in which method the yarn is heated and as the heated yarn enters the balloon it is rotated about its longitudinal axis by sliding over the inner surface of a false-twist annular

body, so as to impart a twist angle to the yarn, characterized in that the distance between the lower portion of the annular false-twist body and the upper portion of the tube on which the yarn is being wound lies between 1 and 10 mms, and the inside diameter of the false-twist annular body varies between 10 mms. greater than and 30 mms less than the outside diameter of the tube on which the yarn is being wound.

2. The method of claim 1 wherein the annular false-twist body engages the yarn with a frictional surface formed of rubber-like material.

3. The method of claim 1 wherein the annular false-twist body engages the yarn with a frictional surface formed of rubber-like material, having a hardness of at least 70 Shore.

4. A method according to claim 1, characterized in that the yarn is a polyamide yarn and the temperature is comprised between 15°C below, and 60°C below the melting point of the yarn.

5. A method according to claim 1, characterized in that the yarn is drawn upstream of the false-twist annular body.

6. A yarn as produced according to the method as claimed in claim 1.

\* \* \* \* \*

30

35

40

45

50

55

60

65